

## UNITED STATES PATENT OFFICE.

HENRY DREYFUS, OF LONDON, ENGLAND.

## MANUFACTURE OF ARTIFICIAL THREADS AND FILAMENTS.

No Drawing. Application filed February 25, 1924, Serial No. 695,117, and in Great Britain March 7, 1923.

This invention relates to the manufacture of artificial silk, artificial horsehair or like threads or filaments from cellulose acetate.

The invention relates especially to the manufacture of such artificial threads or filaments by the dry or evaporative method of formation, that is to say wherein the solutions of or containing the cellulose acetate are extruded through fine orifices into an evaporative atmosphere of air or other gaseous medium (usually heated) in order to form filaments by evaporation of solvent from them, the filaments being usually associated into threads continuously with their production. The invention may also be employed in the manufacture of the threads or filaments by the wet coagulation method, i. e., wherein the solutions are extruded through fine orifices into coagulation or precipitation baths.

In my previous British specification No. 210,108 and U. S. application S. No. 648,350, I have shown that with highly or relatively highly concentrated solutions of cellulose acetate, threads or filaments can be obtained having special properties, being of rounder section, and showing less "glitter" effect.

However, the surprising fact has since been found that the threads so produced, while possessing these advantageous properties, show much less covering power in the form of finished goods such as fabrics, which is a matter of considerable importance from the point of view of the value of such a fibre. The explanation for this may perhaps be that the density of a thread produced from a concentrated solution is increased, and thus gives the disadvantage of lowering the covering power in a fabric, so that it is necessary to use a considerably greater number of threads for a given surface of fabric.

For example, if the concentration of the cellulose acetate solution to be spun is raised to over 20%, e. g. between 20 and 30%, it will be seen that the threads or filaments have less covering power in the measure as the concentration is increased.

It has now been found when employing highly viscous cellulose acetates, having viscosities not less than 50, as hereinafter defined that in proportion as the concentration of the solutions to be spun is decreased, e. g. below 20%, for instance to between 20%

and 10%, or below 10%, for example to 5% or less, the covering power of the threads or filaments obtained is increased, and it is possible in this way to obtain threads of substantially increased covering power. At 60 the same time the form or configuration of the filaments or threads produced is, in spite of the dilution, more round, and "glitter" is avoided. Further it has been found that as the section of the filaments is more 65 round, their liability to become more woolly in character on heating for a long time in water is considerably reduced or even suppressed.

This a very important desideratum in the 70 industry, as the value of an artificial silk or like thread is judged in particular by its covering power reckoned on a certain weight of the given textile thread as compared with others.

For the present invention I employ highly viscous cellulose acetates having viscosities ranging from 50 to 100, 150, 200 or more, reckoned on the basis of an acetone solution of the cellulose acetate containing 6 grams 80 per 100 cc. acetone as compared at 25° C. with the viscosity of pure glycerol taken as 100, in a viscosimeter such for example as the Engler viscosimeter. The viscosities indicated in the claiming clauses hereto are to be 85 understood as reckoned on such basis. These highly viscous cellulose acetates are obtainable by the processes of my British specification No. 207562 and the specification of my corresponding U. S. application 90 Serial No. 633,016, which specifications allow, as therein stated, of producing cellulose acetates of such remarkably high viscosity properties that even solutions of much greater dilution (for example 50% greater 95 dilution or more) made therewith can be just as viscous as much more highly concentrated solutions (for example solutions of 50% greater concentration or more) of 100 my previously known cellulose acetates, obtained for example by the processes of my British specifications 6463 of 1915, 14101 of 1915, 100009 or 101555, which themselves were the most viscous cellulose acetates ever produced before my said British specification 105 No. 207562 or my U. S. application S. No. 633,016. The products of my said last mentioned British specification and U. S. application are moreover characterized by their 110 enormously increased strength in the form

of threads and an enormously increased wet strength of threads made with them, which is the best proof that the cellulose molecule is much more preserved in them.

5 The spinning solutions made with the before mentioned high viscosity cellulose acetates obtainable by the processes of my said British specification No. 207562 and U. S. application S. No. 633,016 may be of concentrations containing less than 20% of the cellulose acetate, and more especially less than about 16%, and particularly concentrations of from about 10% to 5% or less. Any desired solvents may be employed in making 10 the solutions.

15 The following is one example of artificial silk spinning solutions according to the invention, it being understood that this is given only by way of illustration and can be varied 20 considerably. The parts are by weight.

*Example.*

An acetone-soluble cellulose acetate is employed made for example as follows in 25 accordance with my British specification No. 207562 or U. S. application Serial No. 633016.

30 100 parts by weight of cellulose, for example cotton, are introduced into a mixture of about 800 parts by weight of glacial acetic acid, 15-20% of sulphuric acid relatively to the weight of the cellulose (and reckoned on the basis of sulphuric acid of 100% strength), and about 200 to 250 parts 35 by weight of acetic anhydride, this mixture having been first cooled down to 0° C.; the temperature is only allowed to rise gradually, cooling being continued until complete solution, the reaction being continued 40 until a test portion shows that the acetylation product is soluble in acetone, for example about 2 to 6 hours. If desired, the temperature may be allowed to rise to about 25° or 30° C. towards the end of the acetylation. 45 The acetylation product may be isolated in the known way and employed as such, or it may be first submitted to a secondary reaction or treatment, for example by allowing it to stand in the acetylation solution at about ordinary temperature or with slight heating, after, if necessary, adding a 50 small quantity of water or other agent capable of destroying any acetic anhydride remaining, the product being isolated while soluble in acetone.

55 100 parts by weight of the cellulose acetate made as described are dissolved in 900 to 1900 parts of acetone to form the spinning solution.

60 The artificial threads or filaments will usually be produced according to the dry spinning or evaporative method. The threads or filaments produced according to the invention may or may not be subjected 65 to traction in the known way to draw them

out to any desired fineness of denier during their production.

What I claim and desire to secure by Letters Patent is:—

1. A process for the production of cellulose acetate artificial threads and filaments, which comprises spinning said threads and filaments from solutions of cellulose acetates which cellulose acetates have viscosities of not less than 50, reckoned as aforesaid, said spinning solutions being of concentrations between about 4% and 20%. 70

2. A process for the production of cellulose acetate artificial threads and filaments, which comprises spinning said threads and 80 filaments from solutions of cellulose acetates which cellulose acetates have viscosities of not less than 50, reckoned as aforesaid, said spinning solutions being of concentrations between about 5% and 16%. 85

3. A process for the production of cellulose acetate artificial threads and filaments, which comprises spinning said threads and filaments from solutions of cellulose acetates which cellulose acetates have viscosities ranging from 50 to about 200, reckoned as aforesaid, said spinning solutions being of concentrations between about 4% and 20%. 90

4. A process for the production of cellulose acetate artificial threads and filaments, which comprises spinning said threads and filaments from solutions of cellulose acetates which cellulose acetates have viscosities ranging from 50 to about 200, reckoned as aforesaid, said spinning solutions being of 100 concentrations between about 5% and 20%. 95

5. A process for the production of cellulose acetate artificial threads and filaments, which comprises spinning said threads and filaments from solutions of cellulose acetates which cellulose acetates have viscosities ranging from 50 to about 200, reckoned as aforesaid, said spinning solutions being of 105 concentrations between about 5% and 16%. 110

6. Spinning solutions for artificial threads and filaments containing cellulose acetates having viscosities not less than 50, reckoned as aforesaid, said spinning solutions being of concentrations between about 4% and 20%. 115

7. Spinning solutions for artificial threads and filaments, containing cellulose acetates having viscosities not less than 50, reckoned as aforesaid, said spinning solutions being of concentrations between about 5% and 16%. 120

8. Spinning solutions for artificial threads and filaments, containing cellulose acetates having viscosities ranging from 50 to about 200, reckoned as aforesaid, said spinning 125 solutions being of concentrations between about 4% and 20%.

9. Spinning solutions for artificial threads and filaments, containing cellulose acetates having viscosities ranging from 50 to about 200, reckoned as aforesaid, said spinning 130 so.

lutions being of concentrations between about 5% and 20%.

10. Spinning solutions for artificial threads and filaments, containing cellulose acetates having viscosities ranging from 50 to about 200, reckoned as aforesaid, said spinning solutions being of concentrations between about 5% and 16%.

11. Cellulose acetate artificial threads and filaments made from solutions between about 4% and 20% in concentration, of cellulose acetates having viscosities not less than 50 reckoned as aforesaid, said threads and filaments possessing high covering power, high mechanical strength, relatively round filament section and substantial freedom from glitter.

ment section and substantial freedom from glitter.

12. Cellulose acetate artificial threads and filaments made from solutions between about 5% and 16% in concentration, of cellulose acetates having viscosities between 50 and about 200 reckoned as aforesaid, said threads and filaments possessing high covering power, high mechanical strength, relatively round filament section and substantial freedom from glitter.

In testimony whereof I have hereunto subscribed my name.

HENRY DREYFUS.